

## [54] EXPLOSIVE COMPOSITION WITH GROUP VIII METAL NITROSO HALIDE GETTER

[76] Inventors: Franklin E. Walker, 18 Shadow Oak Rd., Danville, Calif. 94526; Richard J. Wasley, 4290 Colgate Way, Livermore, Calif. 94550

[21] Appl. No.: 16,746

[22] Filed: Mar. 2, 1979

## Related U.S. Application Data

[63] Continuation-in-part of Ser. No. 610,166, Sep. 4, 1975, Pat. No. 4,142,927.

[51] Int. Cl.<sup>3</sup> ..... C06B 31/00

[52] U.S. Cl. ..... 149/45; 149/23; 149/24; 149/33; 149/46; 149/61; 149/88; 149/89; 149/92; 149/93; 149/100; 149/101; 149/105; 149/108

[58] Field of Search ..... 149/105-107, 149/36, 45, 23, 24, 33, 46, 61, 88, 89, 92, 93, 100, 101, 108

[56]

## References Cited

## U.S. PATENT DOCUMENTS

|           |         |                        |         |
|-----------|---------|------------------------|---------|
| 3,132,060 | 5/1964  | Beegle et al. ....     | 149/36  |
| 3,265,545 | 8/1966  | Murray ....            | 149/105 |
| 3,536,544 | 10/1970 | Pennington et al. .... | 149/106 |
| 3,706,607 | 12/1972 | Chrisp ....            | 149/36  |
| 3,713,916 | 1/1973  | Braak et al. ....      | 149/105 |
| 4,012,245 | 3/1977  | Voigt et al. ....      | 149/105 |

Primary Examiner—Edward A. Miller

Attorney, Agent, or Firm—Michael D. Nelson

[57]

## ABSTRACT

An improved explosive composition is disclosed and comprises a major portion of an explosive having a detonation velocity between about 1,500 and 10,000 meters per second and a minor amount of a getter additive comprising a non-explosive compound or mixture of non-explosive compounds capable of chemically reacting with free radicals or ions under shock initiation conditions of 2,000 calories/cm<sup>2</sup> or less of energy flu-

ence.

6 Claims, No Drawings

## EXPLOSIVE COMPOSITION WITH GROUP VIII METAL NITROSO HALIDE GETTER

The Government has rights in this invention pursuant to Contract W-7405-ENG 48 awarded by the U.S. Department of Energy.

### RELATED APPLICATIONS

This application is a continuation-in-part of U.S. Ser. No. 610,166 filed Sept. 4, 1975, now U.S. Pat. No. 4,142,927 issued Mar. 6, 1979, which application is incorporated herein by reference.

### BACKGROUND OF THE INVENTION

This invention relates to modifying the explosion performance characteristics of an explosive by doping the explosive with a free radical or ion getter. Typical explosion performance characteristics which may be modified include initiation sensitivity, detonation velocity, brisance, etc. It is believed that under ideal conditions, a typical explosion follows the path shown below:



In the first step (I) a shock wave is applied to the explosive either by a mechanical, vibrational, thermal or electric shock. The non-explosive getter additive of the present invention can increase the amount of shock necessary to initiate the explosion. This is important in formulating explosives since it allows the use of more powerful explosives in conventional applications where the explosives were previously too sensitive.

In the second step (II) the explosive undergoes compression, heat and shear caused from the shock wave. The third step (III) is the generation of free radicals and/or ions. The doping of the explosive with a compound which will capture or deactivate free radicals or ions, the number of initiation sites can be controlled. The number of initiation sites, the fourth step (IV), affects the rate of detonation. Thus, by using the additives of this invention the detonation velocity and brisance can be modified.

The fifth step (V) is the decomposition of the explosive. This decomposition is a function of time and number of initiation sites. Since the number of initiation sites can be varied by the presence of the additive of this invention, and since the number of initiation sites has an effect upon the number of molecular decompositions, the decomposition time can also be modified by the use of the additives of this invention.

The sixth step (VI) is the explosive reaction yielding the high energy release. This explosive reaction is a function of the critical initiation energy of the explosive (See UCRL-75722, Apr. 21, 1975, Lawrence Livermore Laboratory Report by F. E. Walker and R. J. Wasley).

The explosive reaction can also be modified by proper selection of the additive of this invention.

It is an object of this invention to provide an additive which when added to an explosive modified the explosion performance characteristics.

It is an additional object of this invention to provide an improved explosive.

It is a further object of this invention to provide a method for modifying the explosion characteristics of an explosive.

Other additional and further objects will become apparent from the following description of the invention and accompanying claims.

### SUMMARY OF THE INVENTION

The foregoing objects and their attendant advantages can be realized by incorporating into a major portion of an explosive, which is capable of being detonated by a mechanical or electrical shock, a minor portion of a getter additive comprising a non-explosive compound or mixture of non-explosive compounds capable of capturing or deactivating free radicals or ions under mechanical or electrical shock conditions, that is, the compound is capable of chemically reacting with free radicals and/or ions under shock initiation conditions of 2,000 calories/cm<sup>2</sup> or less energy fluence. Exemplary classes of compounds include C<sub>4</sub>-C<sub>32</sub> organic isocyanates, C<sub>2</sub>-C<sub>30</sub> olefins, iodine, C<sub>1</sub>-C<sub>12</sub> organic nitroso hydrocarbons, C<sub>1</sub> to C<sub>12</sub> organo nitroso halides, Group VIII metal nitroso halides, C<sub>2</sub> to C<sub>16</sub> organo hydrazines, and Group IIIB IVA, VIII, VIIB and IVB metal fluorides.

We have discovered that the explosion performance characteristics, i.e. initiation sensitivity, detonation velocity, brisance, etc., of an explosive can be conveniently modified by the use of the non-explosive getter additives of this invention. It is well known that the initiation sensitivity of an explosive is effectively decreased by the addition of a non-explosive diluent. Explosives which detonate under a given set of conditions will generally be less sensitive to detonation upon dilution. The additives of this invention reduce the initiation sensitivity considerably beyond that reduction which would be expected by dilution.

Although not wishing to be bound by the theory, it is believed that the additives of this invention chemically combine and deactivate free radicals or ions under shock conditions thereby depressing the initiation of the explosive reaction. Regardless of the theory or mechanism involved, we have found that the inclusion of the getter additives of this invention to an explosive significantly affects the explosion performance characteristics.

### Explosives

Explosives which may be used in the practice of this invention are metastable chemical compounds that are capable of releasing their chemical energy explosively, i.e., in a very short time, from a mechanical or electrical shock. As referred to herein "mechanical shock" means any sudden change of pressure on the explosive or shearing of the explosive such as occurs from compression by a hammer or the sudden cutting of the explosive with a sharp blade, or by a vibration, etc. The explosives which may be employed typically have a detonation velocity ranging from 1,500 to 10,000 meters per second and more usually from 2,500 to 9,000 meters per second. Exemplary explosives which may be employed

include the nitro aromatic compounds such as trinitrobenzene (TNB), triaminotrinitrobenzene (TATB), diaminotrinitrobenzene (DATB), trinitrotoluene (TNT), trinitroanisole, trinitrocresol, trinitrophenol (picric acid), trinitrophenol, trinitroresorcinol, trinitromethylaniline, diazodinitrophenyl, hexanitrodiphenylamine, hexanitrodiphenyl, diazodinitrophenol, hexanitrodiphenyl sulfide, hexanitrostilbene (HNS), hexanitrodiphenyl sulfone, ammonium picrate, guanidine picrate, benzotrioxadiazole trioxide, etc.; the nitramines such as cyclotrimethylenetrinitramine (RDX), trinitrophenylmethylnitramine (Tetryl), cyclotetramethylenetrinitramine (HMX), ethylenedinitramine, nitroguanidine, etc.; the nitrosamines such as cyclotrimethylenetrinitrosamine, nitrosoguanidine, etc.; the nitric acid esters such as pentaerythritol tetranitrate (PETN), diethanolnitramine dinitrate, nitromannite, nitrostarch, propanetriol trinitrate, diethyleneglycol dinitrate (DEGN), nitrocellulose, nitroisobutyl glycerine trinitrate, tetranitrodiglycerine, nitroglycerol, nitrosugars, glycerine chlorhydrin dinitrate, trimethylolethane trinitrate, nitroglycerine, etc.; other nitro compounds such as tetranitro-2,3,5,6-dibenzo-1,3a,4,6a-tetraazapentalene (TACOT), bis trinitroethylidipate, dinitropropyl acrylate, ethyldinitropentanoate, bis(fluorodinitroethyl) formal, tetranitromethane, nitromethane, amatols, Amatex, etc.; the inorganic nitrates such as ammonium nitrate, barium nitrate, Baratol, potassium nitrate, lead nitrate, etc.; the inorganic azides such as lead azide, silver azide, copper azide, lead dinitrophenylazide, etc.; and other explosives such as lead styphnate, mercury fulminate, lead picrate, lead salts of dinitrosalicylic acid, tetrazene, lead hypophosphate, etc.

The explosives may be in the form of solids, liquids, or gases. They may be used in combinations such as RDX and TNT or individually. Also, liquid explosives may be mixed with solid explosives or gaseous explosives and vice-versa.

Typical detonation velocities are shown in the following table.

TABLE I

| TYPICAL DETONATION VELOCITIES |                      |
|-------------------------------|----------------------|
| Explosive                     | Velocity<br>(m/sec.) |
| Baratol                       | 4800                 |
| Nitrocellulose (13.45% N)     | 7300                 |
| Nitroglycerine                | 7700                 |
| Ammonium nitrate              | 4100                 |
| Trinitrotoluene (TNT)         | 6930                 |
| Picric acid                   | 7000                 |
| Mercury fulminate             | 3920                 |
| Tetryl                        | 7850                 |
| Ammonium picrate              | 6500                 |
| Lead Azide                    | 5000                 |
| HMX                           | 9100                 |
| RDX                           | 8700                 |
| Diaminotrinitrobenzene        | 7520                 |
| Pentaerythritol tetranitrate  | 8260                 |

#### Getter Additives

The getter additives which may be employed in the practice of this invention are compounds either organic or inorganic which are capable of capturing or deactivating (chemically reacting thereby to pair all unpaired electrons and renders ions electroneutral) free radicals or ions under mechanical, electrical or thermal shock conditions but which are not explosives. The higher

molecular weight compounds are preferred such as those having molecular weights between about 80 and 1,000 and more preferably from 125 to 500. The compounds will have the ability to chemically combine with low molecular weight free radicals or ions under shock initiation of 2,000 calories/cm<sup>2</sup> of energy fluence or less. Thus, compounds which are able to deactivate free radicals at 0 energy fluence, such as ambient, quiescent conditions, may be used as getter additives as well as compounds which will deactivate free radicals under shock initiation of 2,000 calories/cm<sup>2</sup> of energy fluence. Usually, the lower the energy fluence necessary in order to activate the getter additive, the better the getter additive in desensitizing the explosive. Depending upon the desired properties, a getter additive capable of capturing more than one free radical and/or ion can be highly advantageous. Getter additives which may be employed to vary the explosion performance characteristics include the following:

20 I. Isocyanates having from 4 to 32 carbons and preferably having at least one carbon-carbon chain longer than 4 carbons and preferably longer than 6 carbons. The isocyanates which may be employed generally have the following formula:



Wherein:

30 R is a hydrocarbylene having from 2 to 30 carbons, preferably from 4 to 15 carbons and more preferably having from 6 to 12 carbons;

x is an integer equal to 0 or 1, preferably 1; and  
y is an integer equal to 0 when x is 1 and equal to 1 when x is 0.

35 As referred to herein hydrocarbylene is a divalent radical composed mostly of hydrogen and carbon and may be aliphatic, alicyclic, aromatic or combinations thereof, e.g., alkylarylene, aralkylene, arylene, alkylene, alkylcycloalkylene, cycloalkylarylene, etc., and may be saturated or unsaturated. Exemplary isocyanates which may be employed are monoisocyanates such as hexylisocyanate, decylisocyanate, dodecylisocyanate phenylisocyanate, tolylisocyanate, cyclohexylisocyanate, xyleneisocyanate, cumeneisocyanate, abietylisocyanate, etc.; diisocyanates such as hexanediisocyanate, decanedediisocyanate, octadecanediisocyanate, phenylenediisocyanate, tolylenediisocyanate, bis(diphenylisocyanate), methylene bis(phenylisocyanate), bis(phenylisocyanate) sulfide, etc.

50 55 Various functional groups may be present on or in the hydrocarbylene chain and may be halo, carbonyl, amido, oxy, alkoxy, epoxy, carboxy, carboxyl, sulfoxyl, sulfonyl, sulfino, sulfo, etc.

II. Olefins having from 2 to 30 carbons and preferably having from 4 to 20 carbons. The olefins may have multiple olefinic bonds and may be conjugated or non-conjugated. Exemplary olefins include, ethylene, propylene, butene, isobutene isoprene, isopentene, cyclohexene, pentadiene, hexadiene, decene, dodecene, octadecene, octadecadiene, phenylpropene, diphenylpropene, etc.

III. Iodine.

60 65 IV. Organo nitroso hydrocarbons having from 1 to 12 carbons and preferably from 4 to 10 carbons. Exemplary nitroso compounds include 2-methyl-2-nitroso propane, nitrosobutane, nitroso propane, nitroso ben-

zene, p-nitrosodimethylaniline, p-nitroso-N-methylaniline, n-nitroso-N-methylaniline, etc.

V. Organo nitroso halides having from 1 to 12 carbons and preferably from 4 to 10 carbons. Exemplary nitroso halides include dichloro nitroso ethane; 1, 2 dibromo, 3 nitroso propane; 1,1 dichloro 4 nitroso butane; 2,5 dichloro 1 nitroso dimethyl aniline, etc.

VI. Organo anhydrides having from 2 to 16 carbons and preferably from 4 to 12 carbons. Exemplary anhydrides include phthalic anhydrides, succinic anhydride, adipic anhydride, diacetyl dibenzoyl anhydride, etc.

VII. Organo nitriles having from 2 to 12 carbons and preferably from 4 to 10 carbons. Exemplary nitriles include ethyl nitrile, propyl nitrile, butyl dinitrile, benzyl nitrile, propylene nitrile.

VIII. Group VIII metal nitroso halides. Group VIII, period V metal nitroso halides are preferred. Exemplary metal nitroso halides are ruthenium nitroso chloride, ruthenium nitroso bromide, rhodium nitroso chloride, ferrous nitroso chloride, nickel nitroso chloride, etc.

IX. Organo hydrazines having from 2 to 16 carbons and more preferably from 4 to 12 carbon atoms. Exemplary hydrazines include dimethyl hydrazine, diethyl hydrazine, dipropyl hydrazine, dibenzyl hydrazine, etc.

X. Group III B, IV A, IV B, VIII or VII B metal fluorides. Any one or more of the metal fluorides falling within, Group III B, IVB IV A, VIII and VII B may be used. Exemplary metal fluorides include scandium fluoride, stannous fluoride, antimony fluoride, manganese fluoride, cobalt fluoride, uranium fluoride, lead fluoride, titanium fluoride, zirconian fluoride, etc.

#### Preparation

The composition of this invention can be prepared by simple admixture of the explosive and the getter additive. The getter additive may be solid, liquid or gaseous. In the event of a solid, the getter additive should preferably be pulverized or otherwise rendered into a powder form and intimately mixed with the explosive. The explosive-additive mixture may then be used directly or 40 slurred, pressed, cast, gelled, extruded, plasticized, pelletized, etc. In one embodiment of the invention, the getter additive is admixed with only a portion of the explosive. It should be recognized that many methods of preparation and design may be utilized within the 45 scope of the present invention.

In the event the getter additive is a liquid, it can be incorporated into the explosive in the same manner as discussed above. If the explosive is a solid, then a paste or slurry of the explosive and getter additive may be made. If the explosive is also a liquid, the two may be used as a liquid mixture or incorporated onto a solid support. Alternatively, the mixture may be thickened into a gel. In still another embodiment, the mixture is polymerized into a polymeric matrix. In this embodiment it may be necessary with some of the additives to add them after polymerization.

In the event the getter additive is a gas, the explosive may be used in the gaseous state. Alternatively, the getter additive may be dissolved in a carrier liquid or in the explosive. In still another embodiment, a gas precursor may be employed which releases the gaseous getter additive prior to use or detonation.

The amount of getter additive which may be employed in the practice of this invention can vary over a wide range depending upon the type of explosives involved, the type of getter additives selected, etc. Generally, however, the getter additive will be present in an

amount from 0.01 to 20 percent by weight of the final explosive and preferably will be present in an amount from 0.2 to 10 weight percent.

The weight ratio of getter additive to explosive will generally vary from 0.01 to 20 weight parts of getter additive for each 100 weight parts of final explosive and preferably from 0.2 to 10 weight parts of getter additive for each 100 weight parts of final explosive.

It should be recognized that precursors of the getter additives may be prepared and added to the explosive and such precursors are included within the scope and spirit of this invention. It is also recognized that compounds other than the classes specifically set forth in the specification may be employed provided that such compounds are capable of capturing free radicals or ions under shock conditions and are not explosive themselves. An additive is classified as a non-explosive if it cannot be exploded by a mechanical shock and has a detonation velocity below 1,500 meters per second. A mechanical shock for purposes of determining whether a substance is classified as a non-explosive is defined as that which transfers not less than 2,500 cal/cm<sup>2</sup> of energy fluence.

#### Other Additives

In addition to the getter additive of this invention, other additives may be present without adversely affecting the getter's performance properties. Exemplary additives include oxidizers such as metallic nitrates, e.g., sodium, and potassium nitrate, etc.; swelling agents such as guar flour, cellulose, carboxymethyl cellulose, etc.; powdered metals such as aluminum, magnesium, zirconium, titanium, etc.; polymers such as vinyl, acrylic and alkylene oxide polymers, PVA, polyacrylamide, etc.; alkali metal azides such as sodium and potassium azide, etc.; water; carbonaceous materials such as powdered coal, fuel oil, coal dust, charcoal, wood meal, etc.; glass powder and others.

The amount of other additives which may be employed may vary over a wide range depending upon the type of additive selected, the purpose, the type of explosive, etc. Generally, however, the other additives will be present in an amount varying from 0 to 60 percent but usually varying from 0.1 to 30 percent and more usually varying from 1 to 20 percent by weight of the total composition.

#### Uses

The explosive compositions of this invention can be used in a wide variety of applications. They may be used in typical demolition and blasting activities, in well fracturing (See U.S. Pat. No. 3,825,452), in making molded explosives of varying detonation speeds (See U.S. Pat. No. 3,619,306), in generating gases such as nitrogen for use in dynamic lasers (See U.S. Pat. No. 3,773,947), or for use in automobile crash bags (See U.S. Pat. No. 3,785,674), in making rocket fuels (See U.S. Pat. No. 3,804,683), in making ammunition (See U.S. Pat. No. 2,111,203), in making fuses (See U.S. Pat. No. 3,421,441), in welding (See U.S. Pat. No. 367,234), in bombs and many other applications.

The composition of this invention may also be employed in making armor-piercing bombs and rockets.

The following examples are presented to illustrate the practice of specific embodiments of this invention and should not be interpreted as limitations upon the scope of the invention.

## EXAMPLE 1

This example is presented to illustrate the initiation sensitivity of an explosive. In this test, a compression wave of varying strengths is applied to a sample explosive by impacting a weight against the sample until the explosive detonates (explodes).

This test is typically called the drop hammer test. The drop hammer test is more fully described in the Manual for Sensitiveness Tests, TTCP Panel 0-2, February 1966, Canadian Armanent Research and Development Report, which is herein incorporated by reference. Briefly, a 2.5 kilogram hammer is guided to various heights above a 1½ inch diameter 10 inch high cylindrical steel striking pin (weight is 2.5 kilograms). The striking pin rests on the sample explosive which in turn rests on a hardened steel anvil.

The test sample of approximately 35 mg. is placed on 80-100 mesh sand paper which rests on the anvil and the striking pin is gently pressed down upon the sample. The hammer is dropped from a given height onto the striking pin. If no explosion occurs, the test is repeated with a fresh sample from successively greater heights until an explosion occurs. If an explosion occurs, a fresh sample is replaced in the test machine and tested at successively lower heights until a point of no explosion is reached. Thereafter, a sample is tested at a given increment below the level at which the previous sample was tested if that sample exploded, and at a given increment above the level which the previous one was tested if it did not explode. By using this up-and-down method and analyzing the data statistically, a height for 50% ignition probability is attained. The procedure for determining this height and the error at a 95% confidence level is discussed by W. J. Dixon and A. M. Mood, "Method of Obtaining and Analyzing Sensitivity Data", *Journal American Stat. Assoc.*, Vol 43, 1948, pp 109-126, which is herein incorporated by reference.

A microphone is mounted on the anvil face and the signal from the microphone is fed to an amplifier which in turn triggers a thyratron tube. Triggering the thyratron tube lights a neon lamp on the panel. This indicates whether the sample exploded.

The following table illustrates the ignition sensitivity for various commercial explosives.

TABLE II

| Drop Hammer Height    |         |
|-----------------------|---------|
| Trinitrotoluene (TNT) | 100 cm. |
| HMX                   | 39 cm.  |

## EXAMPLE 2

This example illustrates the desensitizing effect of a non-explosive diluent on the ignition sensitivity. An approximate 2 gram portion of TNT is added to a small 50 cc glass bottle and about 100 milligrams of benzoic acid are added. The bottle is tumbled for about 30 minutes to uniformly mix the explosive with the diluent. Thereafter successive 35 milligram portions of the mixture are tested in the drop hammer test. The results show that the addition of 5 percent of a diluent increased the drop hammer height to about 145 cm.

## EXAMPLE 3

This example is presented to illustrate that mixtures of explosives do not automatically change the ignition sensitivity. The same procedure as discussed in Exam-

ple 2 is followed except that 5 percent of HMX is mixed with 95% of TNT and no additives were added. The sample exploded at 100 cm.

## EXAMPLE 4

The procedure of Example 2 is repeated except that phthalic anhydride diluent is used instead of benzoic acid. The Sample of 95% TNT and 5% phthalic anhydride exploded at about 145 cm.

## EXAMPLE 5

This example is presented to illustrate the reduction in ignition sensitivity by the addition of a non-explosive free radical or ion getter to the explosive. In this test, approximately 2 grams of TNT fine powder are placed in a 50 cc glass bottle along with about 100 milligrams of tolylene diisocyanate. The bottle is tumbled for about 10 minutes to uniformly mix the explosive and the additive. Next, successive 35 mg. portions of the mixture are tested in the drop hammer apparatus. The mixture did not explode even when the highest position on the drop hammer apparatus was used, i.e. 177 cm.

## EXAMPLE 6

The procedure of Example 5 is repeated except that azo bis isobutryldiisocyanate is used in place of the tolylene diisocyanate. The explosive mixture exploded at 155 cm.

## EXAMPLE 7

The procedure of Example 5 is repeated except that Iodine is used in place of the tolylene diisocyanate and only 40 milligrams was used. The mixture of 98% TNT and 2% of Iodine exploded at 141 cm. TNT with a diluent at 2% is believed to explode at 114 cm according to extrapolation.

## EXAMPLE 8

The procedure of example 5 is repeated except that carbon tetrachloride is used in place of the tolylene diisocyanate. The explosive mixture would not explode when the drop hammer is raised to its highest point on the machine of 177 cm.

## EXAMPLE 9

The procedure of Example 5 is repeated except that dimethyl hydrazine is used in place of tolylene diisocyanate. The explosive mixture exploded above 158 cm in drop hammer height.

## EXAMPLE 10

The procedure of Example 5 is repeated except that azo-bis-isobutyl dinitrile is used in place of tolylene diisocyanate. The mixture exploded when the drop hammer was raised to 155 cm.

TABLE III

| DROP HAMMER TEST |           |                          |             |
|------------------|-----------|--------------------------|-------------|
| Example          | Explosive | Additive                 | Height (cm) |
| 1.               | TNT       | none                     | 100         |
| 2.               | TNT       | Diluent*                 | 145         |
| 3.               | TNT & HMX | none                     | 100         |
| 4.               | TNT       | Diluent**                | 145         |
| 5.               | TNT       | Tolylene<br>Diisocyanate | 177         |
| 6.               | TNT       | ABID***                  | 155         |
| 7.               | TNT       | Iodine (2%)              | 141         |
| 8.               | TNT       | Carbon Tetraiodine       | 177         |
| 9.               | TNT       | Dimethyl Hydrazine       | 158         |
| 10.              | TNT       | azo-bis-isobutyl         |             |

TABLE III-continued

## DROP HAMMER TEST

| Example | Explosive | Additive | Height (cm) |
|---------|-----------|----------|-------------|
|         | dinitrile |          | 155         |

\*Diluent used was benzoic acid

\*\*Diluent was phthalic anhydride

\*\*\*ABID is azo-bis-isobutyryldiisocyanate

## EXAMPLE 11

This test is presented to measure the velocity of the shock wave. A getter additive will reduce the velocity. The reduction in velocity will increase the transit time. Hence, a getter additive will increase the transit time. The test is called the Gas Gun Initiation Test and is a standard test recognized in the explosives community.

The test is run by firing a sabot (a free floating support for a projectile) with a thin flyer plate mounted on the forward portion thereof. The sabot is guided by a gun muzzle which delivers or guides the sabot to a target. The target is the test explosive. This test explosive has a flat face which is positioned so as to come into uniform contact with the flyer plate. The opposite side of the test explosive or target is tiered. There is a row of crystal pins mounted on each tier to give precise arrival time of the shock wave at each tier. The shock transit time is measured across the tiered explosive.

The composition and velocity of the flyer plate are known so as to yield a known kinetic energy for the plate. The explosive mixture is pressed and machined into the tiered shape. The Sabot is fired from the gas gun against the test sample and the shock travel time is measured by electronic data taken from the crystal pins. A computer calculates the shock velocity and excess transit time.

The test is conducted with TNT alone, with TNT (95%) and an inert diluent of  $\text{SiO}_2$  (5%) and with TNT

(95%) and Ruthenium nitroso chloride  $\text{Ru}(\text{NO})_2\text{Cl}_2$  (5%). The results of the test are as follows:

TABLE IV

| GAS GUN TEST |                                           |                    |
|--------------|-------------------------------------------|--------------------|
| Test         | Explosive                                 | Transit Time (sec) |
| 1.           | TNT - Control                             | 0.37               |
| 2.           | TNT + $\text{SiO}_2$                      | 0.39               |
| 3.           | TNT + $\text{Ru}(\text{NO})_2\text{Cl}_2$ | 0.54               |

The above table illustrates the dramatic effect of the getter additive on the explosion characteristics of an explosive. The increase in transit time by the use of Ruthenium nitroso chloride illustrates a reduction in decomposition rate of the explosive.

We claim:

1. A composition of matter comprising a major portion of a metastable explosive capable of being detonated by a mechanical, electrical or thermal shock and having a detonation velocity between about 1,500 and 10,000 meters per second and a minor amount of a getter additive comprising a Group VIII metal nitroso halide.

2. The composition defined in claim 1 wherein said getter additive is present in an amount from 0.01 to 20 weight percent.

3. The composition defined in claim 1 wherein said getter is a Group VIII metal nitroso chloride.

4. The composition defined in claim 3 wherein said getter additive is ruthenium nitroso chloride.

5. The composition defined in claim 1 wherein said explosive is selected from trinitrotoluene, cyclotrimethylenetrinitramine, trinitrophenylmethylnitramine, triamino trinitrobenzene, pentaerythritol tetranitrate, diaminotrinitrobenzene, ammonium nitrate, nitroguanidine and diethyleneglycol dinitrate.

6. The composition defined in claim 1 wherein said explosive is trinitrotoluene and said getter is ruthenium nitroso chloride.

\* \* \* \* \*